

July 20, 1971

TSUNEO SUGA ET AL

3,594,173

LITH-TYPE PHOTOGRAPHIC MATERIAL

Filed Oct. 30, 1968



## 1

3,594,173

**LITH-TYPE PHOTOGRAPHIC MATERIAL**  
 Tsuneo Suga, Akio Oshima, and Yuji Kuroda, Tokyo,  
 Japan, assignors to Konishiroku Photo Industry Co.,  
 Ltd., Tokyo, Japan

Filed Oct. 30, 1968, Ser. No. 771,807

Claims priority, application Japan, Oct. 31, 1967,  
 42/69,710

Int. Cl. G03c 1/28

U.S. Cl. 96—108

3 Claims

**ABSTRACT OF THE DISCLOSURE**

The joint use of certain pyrazolone compounds together with a gold sensitizer is found to be particularly effective 15 to obtain a lith-type silver halide photographic emulsion improved in high-intensity reciprocity failure. The pyrazolone compound has the general formula:



wherein R is an acylamino, arylamino, alkyl, aryl or 30 aralkyl group and X is a hydrogen atom, halogen atom, carboxyl, sulfone, phenoxy amino or nitro group.

This invention relates to a light-sensitive silver halide 35 photographic material. More particularly, the present invention is concerned with a light-sensitive silver halide photographic material useful for halftone reproduction (this is referred to as a lith-type film hereafter). It is an object of the invention to provide a lith-type film which 40 is improved in high-intensity reciprocity failure.

As a general rule, the amount of exposure when a light-sensitive photographic material is subjected to exposure can be expressed as the product of light intensity and exposure time. Accordingly, if the light intensity is great 45 as ten times of its original intensity is used, the exposure time can be decreased to one-tenth its original time thereby to obtain the original result. Usual photo-snapping is conducted according to the above relationship by adjusting a diaphragm value and an exposure time. However, when light intensity is extremely large or small, the deviation of photographic characteristics occurs even at the same exposure amount. For example, the decrease in photographic speed is observed when exposure at high intensities for a short exposure time or at low intensities for a long exposure time is made. This phenomenon is well known as reciprocity law failure.

A lith-type film also suffers from the above phenomenon. Further, lith-type film is usually required to be treated with an infectious developer having a low sulfite ion concentration and containing hydroquinone, because high image contrast and sharp halftone dots are desired. If the lith-type film is treated with the infectious developer, much more reciprocity law failure occurs in comparison with the treatment with a usual developer (methoxyhydroquinone). Particularly, reciprocity law failure is severe at high intensities. For example, when exposure is conducted at a gradually decreased exposure time of 10, 10<sup>-1</sup>, 10<sup>-2</sup>, 10<sup>-3</sup>, 10<sup>-4</sup> and 10<sup>-5</sup> seconds at the correspondingly gradually increased intensities, the image density of 70 photographs obtained by the same development remarkably decreases.

## 2

As is known, a flask light source having an exposure time as short as 10<sup>-3</sup> seconds has been adopted in the graphic art in view of the improvement in operative efficiency. Thus, a lith-type film suited for light exposure at high intensities for a short exposure time is very useful in the current graphic art.

The present invention provides a lith-type film suited for the objects indicated hereinbefore.

The present invention is related to a light-sensitive silver halide photographic material of the lith-type, characterized by that a pyrazolone compound of the general formula



(wherein R represents an acylamino, arylamino, alkyl, aryl or aralkyl group and X represents a hydrogen atom, halogen atom, carboxyl, sulfone, phenoxy, amino or nitro group) and a gold sensitizer are incorporated in the emulsion layer or a layer adjacent thereto.

Typical pyrazolone compounds of the above general formula are listed below:

(1)



(2)



(3)



(4)





3



5



10



15



20



25



30



4



10



15



20

The pyrazolone compounds used in this invention are not limited to those given above.

As gold compounds, the following compounds are used:

- 25 (1) Chloroauric acid -----  $\text{HAuCl}_4$   
 (2) Potassium chloroaurate -----  $\text{KAuCl}_4$   
 (3) Auric trichloride -----  $\text{AuCl}_3$   
 (4) Potassium auric thiocyanate -----  $\text{KAu}(\text{CNS})_4$   
 30 (5) Potassium iodoaurate -----  $\text{KAuI}_4$   
 (6) Tetracyanoauric acid -----  $\text{HAu}(\text{CN})_4$   
 (7) Ammonium aurothiocyanate -----  $\text{NH}_4\text{Au}(\text{CNS})_2$   
 (8) Diethylmonobromogold -----  $\text{Au}(\text{C}_2\text{H}_5)_2\text{Br}$   
 (9) Pyrazolonechlorogold -----  $(\text{C}_5\text{H}_5\text{N})\text{AuCl}_3 \cdot \text{HCl}$

35 In addition, all of gold compounds used as gold sensitizers for ordinary light-sensitive silver halide photographic materials are also effective in this invention.

Single use of each of the compounds in this invention is very insufficient to decrease high-intensity reciprocity failure resulting from infectious development.

This invention is based on the observation that, as evidently illustrated in the examples below, reciprocity law failure at high intensities is significantly improved by jointly incorporating both of the above compounds.

45 The amount of these compounds is variable according to the class belonging to and preferable amount of the pyrazolone compound is from 5 mg. to 10 g. per mol of silver halide and the gold compound is preferably used in an amount of 0.1–100 mg. calculated on the basis of 50 gold atom per mol of silver halide. These compounds may be dissolved in any suitable solvent such as water, alkali, methanol, etc. and be added at any stage of silver halide formation, ripening and pre-coating. Alternatively, these 55 compounds can be added to a layer adjacent to the emulsion layer, such as protective layer or inter layer as well as emulsion layer.

The compounds of the present invention are applicable to the photographic emulsion which has been sensitized by chemical sensitization, for example, sulfur- or reduction- 60 sensitization or by optical sensitization and which has been added with an additive such as hardening agent or coating aid.

The lith-type film according to this invention is characterized by considerable improvement in high-density reciprocity failure and accordingly in density decrease due to intermittent exposure.

The present invention is illustrated in detail by way of the following examples.

#### EXAMPLE 1

To a silver chlorobromide emulsion containing 20 mol percent of silver bromide was added each compound indicated in the Table 1 below. Each emulsion was subjected to ripening at 55° C. for 60 minutes and thereafter 75 added with chrome alum as a hardening agent and saponin

